

## UNITED STATES PATENT OFFICE.

CHARLES W. ADAMS, OF SAGINAW, MICHIGAN, ASSIGNOR TO THE UNITED STATES GRAPHITE COMPANY, OF SAGINAW, MICHIGAN, A CORPORATION OF MICHIGAN.

## GRAPHITIC BEARING.

No Drawing.

Application filed February 1, 1924. Serial No. 690,048.

The object of my invention is to provide a graphitic bearing of relatively great strength combined with a much lower friction coefficient than has heretofore been characteristic of reasonably strong graphitic bearings. My improved bearing is of special value for thrust bearings, which may be in ring form or other suitable form.

I have discovered that a mechanically strong graphitic bearing of low friction coefficient can be produced in the following way:

I take mined graphite ore which is amorphous and which also contains a certain percentage of ash to give strength, but it is important that this ash content shall also be amorphous. The amount of amorphous ash may be in the neighbourhood of 10 per cent or over. For example I have used with success, an amorphous graphitic ore analyzing something over 82 per cent graphitic carbon, with about eight per cent silica and about 4½ per cent alumina, and small percentages or traces of other matters, such as moisture, volatile matter, calcium oxide, etc.

This amorphous graphitic ore, finely pulverized is thoroughly mixed with equally finely pulverized petroleum coke and then a bonding agent, such as crushed coal tar pitch added. Thereupon to the mixture there is added a solvent for the pitch. This solvent may be benzol or naphtha or other such coal-tar derivative, sufficient of this solvent being used to dissolve the pitch and make a homogeneous mixture in the form of a plastic mass when stirred in a mixer.

The product is then dried and re-pulverized, after which the powdery mixture may be pressed into the desired shape, as by a hydraulic press under a pressure of from five to twenty tons per square inch.

The pressed pieces are baked at a temperature which may range from about 750° C. to 1500° C., and are then ready for use, and as I have said, I have found these bearings strong and lubricative without abrasion.

The proportions of the coke, graphite and pitch may be in three substantially equal parts, although I prefer to use a larger percentage of coke and a smaller percentage of the bonding agent.

The term "amorphous graphite" is used in this specification to designate those finely divided graphite ores which exhibit no semblance of crystalline structure. The ash in such ores is equally finely divided, but by the term "amorphous ash" I do not wish to exclude the possibility that such ash or some of it may tend to recrystallize under the heat treatment I have described.

I claim as my invention:

1. A graphitic bearing, consisting of a baked mixture of petroleum coke and graphite and a coal tar derivative, the graphite being amorphous and containing a substantial per cent of amorphous ash.

2. The method of producing a graphitic product which comprises intimately commingling finely divided graphite and petroleum coke with coal tar in the presence of a volatile solvent for the latter, to form a paste in which the graphite, coke and tar are present in substantially equal proportions, but the coke somewhat predominating over the tar, drying the mixture, pulverizing the dried mass, subjecting the dried, pulverized mass to heavy pressure, and baking the latter at a temperature of at least 750° C.

In testimony whereof I have signed my name to this specification.

CHAS. W. ADAMS.